# EUROPEAN PATENT SPECIFICATION

(11) **EP 0 547 100 B1**
(45) Date of publication and mention of the grant of the patent: **22.02.1995**
(21) Application number: 91915560.6
(22) Date of filing: 21.08.1991
(51) Int. Cl.: D21C 9/02, D21C 9/10

(54) **PROCESS FOR TREATMENT OF LIGNOCELLULOSIC PULP AND APPARATUS FOR PERFORMANCE OF THE PROCESS**
HERSTELLUNGSVERFAHREN VON LIGNOZELLULOSISCHEM ZELLSTOFF UND VORRICHTUNG ZUR DURCHFÜHRUNG DES VERFAHRENS
PROCEDE DE TRAITEMENT DE LA PATE LIGNOCELLULOSIQUE ET APPAREIL PERMETTANT DE REALISER CE PROCEDE

(30) Priority: 24.08.1990 DK 2034/90
(43) Date of publication of application: 23.06.1993
(73) Proprietor: NOVO NORDISK A/S, 2880 Bagsvaerd (DK)
(72) Inventor: PEDERSEN, Lars, Saaby, DK-2880 Lyngby (DK)
(74) Representative: Bach, Niels
(86) International application number: DK9100239
(87) International publication number: WO9203608

(56) References cited:
- EP-A- 373 107
- EP-A- 383 999

## Description

A common stage in the treatment of wood chips for paper production is chemical pulping, e.g. the so-called kraft process which is an alkaline sulphate cooking of the wood chips. The native wood chips contain around 30% lignin, and at the end of the chemical cooking process less than 5% of the lignin compounds is still left in the pulp. Due to the strong brown color of the remaining lignin and its tendency to darken in UV light or by oxidation this has to be removed in order to obtain a white pulp without the tendency to color reversion. After the sulphate cooking a multistage washing of the unbleached kraft brown stock takes place. The well washed brown stock can then be treated with an enzyme preparation followed by a subsequent wash before entering the bleach plant.

The invention comprises an improvement of this conventional multistage washing of the unbleached kraft brown stock, followed by the enzyme treatment with the subsequent wash, whereby this improvement is a modification, which improves the economy and facilitates the processing.

After a multistage washing of the unbleached kraft brown stock followed by an enzyme treatment with the subsequent wash the brown color can be removed by a multistage bleaching using e.g. chlorine and/or chlorine dioxide. Due to the ever increasing environmental concern, the dosage of chlorine and/or chlorine dioxide has to be kept at a minimum, and it is for that reason that the enzymatic treatment of the kraft cooked pulp has been introduced, vide e.g. The third International Conference on Biotechnology in the Pulp and Paper Industry, Stockholm, 16-19.6, 1986, page 67-69.

Thus, the sequence of the prior art processes in regard to paper pulping is the following:
1) kraft cooking of the wood chips,
2) multistage washing of the unbleached kraft brown stock
3) enzymatic treatment of the washed brown stock
4) bleaching.

The invention comprises the above indicated processes 2) and 3) and is an improvement thereof, as explained in more detail in the following.

Hitherto the multistage washing of the unbleached kraft brown stock has been performed as indicated on the flow sheet of Fig. 1. In addition to the process stages indicated on Fig. 1 an oxygen delignification stage with subsequent washing may be included either before or after the enzyme stage. This prior art process with an enzyme treatment introduced between the cooking and the bleaching sections exhibits the serious drawback that the enzyme stage includes a washing stage, which is a unit operation that represents a large capital investment.

Thus, the purpose of the invention is the provision of a process for treatment of lignocellulosic pulp which requires a less expensive apparatus or stated otherwise the provision of a reduction of the price of the prior art method for treatment of lignocellulosic pulp comprising a multistage washing of the unbleached brown kraft stock with subsequent enzyme treatment, washing and bleaching, and a corresponding apparatus for performance of the process.

Now, according to the invention it has been found that the purpose of the invention can be fulfilled, if the enzymatic treatment with the subsequent wash is abandoned altogether and the enzymatic treatment is introduced between two brown stock washing units in the multistage washings of the unbleached kraft brown stock, or stated otherwise if the enzyme treatment is introduced upstream the prior art position of the enzyme treatment in the multistage washing, in such manner that the multistage washing for washing out of impurities from the kraft cooking and washing out of the residues from the enzyme treatment is combined.

Thus, the process for treatment of lignocellulosic pulp according to the invention comprising a multistage washing of the unbleached kraft brown stock and a treatment with a xylanase with high pH activity and stability and high heat stability is characterized by the fact that the xylanase treatment is introduced between two brown stock washing units in such manner that the washed stock from the outlet side of one or more of the washing units is transported to a holding tank, that the xylanase with high pH activity and stability and high heat stability is added directly upstream the holding tank, and that the enzyme treated stock is passed further on in the process to the next washing unit. Also in relation to the process according to the invention (Fig. 2) another non-chlorine bleaching stage, e.g. an oxygen delignification stage or an ozone stage may be included either before or after the enzyme stage.

By comparison of Fig. 1 (prior art) and Fig. 2 (invention) it clearly appears that the invention requires one washing unit less than the prior art process, and thus, the process according to the invention fulfils the purpose of the invention. Furthermore, as the tank on Fig. 1 used for the enzyme treatment normally also serves as buffer tank between the kraft cooking and the bleaching plant the residence time of the pulp in the tank often varies within a wide range, e.g. between 30 minutes and 24 hours. In the invention the tank is an integrated part of the washing process. It only serves the need for holding time for the enzyme treatment, which makes it much easier to control the enzyme treatment time. Finally, the invention provides a much better connection to the existing wash water streams. The entire amount of wash water obtained in the process according to the invention will end up in the recovery system for the kraft cooking process, which means that everything that is solubilized during the enzyme treatment will be burned in the recovery boiler whereby the BOD₅ load from the enzyme stage on the effluent streams is eliminated. This is not the case in the prior art system. In the prior art system the wash water from the washing stage after the enzyme treatment normally has to be sewered. The enzyme treatment according to the invention also releases more cooking chemicals from the pulp than a conventional wash with water. This makes it possible to obtain an even better recovery of cooking chemicals than normally obtained.

The three washing units on Fig. 2 are not limiting to the invention, but just an example. Each single unit can represent more than one washing stage. With three washing units one, two or three enzyme treatment units can be introduced according to the invention; just one enzyme treatment unit is shown on Fig. 2.

The bleach boosting effect is measured as the kappa number reduction of pulp after an enzyme treatment followed by a C/D-E bleaching compared to a control which is treated in the same way but without addition of enzyme: (Bleach boosting Effect = Kappa number after C/D-E bleaching of enzyme treated pulp minus kappa number after C/D-E bleaching of pulp treated without enzyme).

Also, the invention comprises an apparatus for performance of the process according to the invention. The apparatus according to the invention is characterized by the fact that a holding tank with piping with facilities for introduction of enzyme is introduced downstream one or more of the washing units except for the last washing unit, that piping is provided for further transport of the stock to the next washing unit, and that the conventional enzyme treatment unit downstream the washing unit is abandoned.

It is to be understood that at least one holding tank with accessories is introduced, and that the maximum number of holding tanks with accessories which can be introduced into the sequence according to the invention equals the number of washing units in the multistage washing process minus 1.

The following example illustrates the invention in comparison to prior art.

### EXAMPLE 1

In order to illustrate the invention an unbleached and unwashed softwood pulp identified as P was washed in one stage as follows:

The pulp P was diluted with fresh water to a consistency of 1% DS and then reconcentrated to a consistency of approximately 20% on a wire screen. This washing sequence is the standard washing stage used throughout this example.

After the washing the pH of the pulp was 9.7.

This pulp sample was divided into two halves.

The first half of this one stage washed pulp was xylanase treated under the following conditions without pH adjustment prior to the enzyme addition.

| | |
|---|---|
| Temperature | 70°C |
| pH | 9.7 |
| Consistency | 10% |
| Time | 3 hours |
| Xylanase | *Streptomyces olivochromogenes*, vide Example 6 in WO-A-91/02839 |
| Enzyme dosage | 5000 EXU/kg dry pulp |

The definition of the EXU xylanase activity unit appears from AF 293.9/1, obtainable on request from NOVO NORDISK A/S, Novo Allé, DK-2880 Bagsvaerd, Denmark.

The xylanase stage was carried out as follows. The pulp was diluted to the desired consistency by addition of fresh water. The enzyme solution was added and mixed into the pulp by vigorous mixing. The pulp was then placed in a water bath to ensure constant temperature for the remainder of the treatment time. The pulp was not mixed during the three hours of holding time.

After the enzyme stage the pulp was carried through two standard washing stages. This pulp sample which was enzyme treated between the first and the second washing stage, was carried out according to the invention and will be referred to later as **inv 1-2**.

The second half of the one stage washed pulp was carried through another standard washing stage. After washing the pH of the pulp suspension was 8.7.

This two stage washed pulp was enzyme treated without pH adjustment prior to the enzyme addition under the following conditions:

| | |
|---|---|
| Temperature | 70°C |
| pH | 8.7 |
| Consistency | 10% |
| Time | 3 hours |
| Enzyme | *Streptomyces olivochromogenes*, vide Example 6 in WO-A-91/02839 |
| Enzyme dosage | 2000 EXU/kg dry pulp |

The enzyme treatment was carried out as described above.

After the enzyme stage the pulp was carried through one standard washing stage. This sample of pulp, which was enzyme treated between the second and third washing stage, was carried out according to the invention and will be referred to later as **inv 2-3**.

In order to illustrate the corresponding prior art the pulp P was first carried through three standard washing stages. Then the pH of the pulp was lowered to 6.5 by addition of sulfuric acid and an enzyme stage was carried out under the following conditions.

| | |
|---|---|
| Temperature | 50°C |
| pH | 6.5 |
| Consistency | 10% |
| Time | 3 hours |
| Enzyme | Pulpzyme™HA |
| Enzyme dosage | 275 FXU/kg dry pulp |

The definition of FXU xylanase activity unit appears from AF 293.6/1, obtainable on request from NOVO NORDISK A/S, Novo Allé, DK-2880 Bagsvaerd, Denmark.

The enzyme treatment was made as described above.

After the enzyme stage the pulp was washed in an extra standard washing stage according to the prior art. This pulp sample will be referred to later as **prior**.

The above experiment used to illustrate prior art was repeated except that no enzyme was added. This experiment served as a control to demonstrate that the enzyme stage really has an effect on the pulp and will be referred to later as **control**.

The xylanases used in this example were selected according to their pH optimum in relation to the pH of the pulp.

After enzyme treatments and washings all the pulps were bleached according to the same two stage bleaching sequence (D50 C50) E.

The bleachings were carried out under the following conditions:

### (D50 C50):

| | |
|---|---|
| Temperature | 50°C |
| Consistency | 5% |
| Time | 20 minutes |
| active Cl dosage | 5.7% (w/w) on dry pulp |

### E:

| | |
|---|---|
| Temperature | 60°C |
| Consistency | 10% |
| Time | 1 hour |
| NaOH dosage | 4.2% (w/w) on dry pulp |

After the bleaching the kappa number of all four pulps were determined.

### Results

| Kappa number of the pulps after the (D50 C50) E bleachings: | | |
|---|---|---|
| | Kappa number | delta Kappa number % |
| Control | 2.85 | - |
| Prior | 2.52 | 11.6 |
| inv 1-2 | 2.50 | 12.3 |
| inv 2-3 | 2.31 | 19.0 |

It is observed that the kappa number of the enzyme treated pulps are reduced compared to the control. This demonstrates that the enzyme treatment in all three sequences, the prior art and the two inventive sequences, has shown a bleach boosting effect.

It is also seen that the kappa numbers obtained by the two sequences carried out according to the invention are lower than the kappa numbers for the prior art sequence.

This demonstrates that the sequence described by the invention besides giving the technical advantages of avoiding one washing unit gives just as good a kappa number reduction or even a better kappa number reduction as the prior art sequence.

## Claims

1. Process for treatment of lignocellulosic pulp comprising a multistage washing of the unbleached kraft brown stock and a treatment with a xylanase with high pH activity and stability and high heat stability, characterized by the fact that the xylanase treatment is introduced between two brown stock washing units in such manner that the washed stock from the outlet side of one or more of the washing units is transported to a holding tank, that the xylanase with high pH activity and stability and high heat stability is added directly upstream the holding tank, and that the enzyme treated stock is passed further on in the process to the next washing unit.

2. Apparatus for performance of the process according to Claim 1, characterized by the fact that a holding tank with piping with facilities for introduction of enzyme is introduced downstream one or more of the washing units except for the last washing unit, that piping is provided for further transport of the stock to the next washing tank, and that the conventional enzyme treatment unit downstream the washing unit is abandoned.

## Patentansprüche

1. Verfahren zur Behandlung von lignocellulosischem Faserbrei, umfassend ein mehrstufiges Waschen von ungebleichtem braunem Kraftpapierrohstoff und eine Behandlung mit einer Xylanase mit einer Aktivität und Stabilität bei hohem pH-Wert und einer hohen Wärmestabilität, gekennzeichnet durch die Tatsache, daß die Xylanasebehandlung zwischen zwei Wascheinheiten des braunen Papierrohstoffs in einer solchen Weise eingeführt wird, daß der gewaschene Papierrohstoff von der Auslaßseite einer oder mehrerer Wascheinheiten in einen Lagertank transportiert wird, daß die Xylanase mit einer Aktivität und Stabilität bei hohem pH-Wert und einer hohen Wärmestabilität direkt stromaufwärts von dem Lagertank zugegeben wird und daß der mit dem Enzym behandelte Papierrohstoff im Verfahren weiter zur nächsten Wascheinheit geleitet wird.

2. Vorrichtung zur Durchführung des Verfahrens nach Anspruch 1, gekennzeichnet durch die Tatsache, daß ein Lagertank mit Rohrleitungen mit Einrichtungen zur Einführung von Enzym stromabwärts von einer oder mehreren Wascheinheiten mit Ausnahme der letzten Wascheinheit eingeführt wird, daß Rohrleitungen zum weiteren Transport des Papierrohstoffs zum nächsten Waschtank bereitgestellt werden und daß die herkömmliche Enzymbehandlungseinheit stromabwärts von der Wascheinheit weggelassen wird.

## Revendications

1. Procédé de traitement d'une pâte lignocellulosique comportant un lavage en plusieurs étapes de pâte kraft brune non-blanchie et un traitement à l'aide d'une xylanase ayant une activité et une stabilité à pH élevé et une stabilité à température élevée, caractérisé en ce que le traitement à la xylanase est introduit entre deux unités de lavage de pâte brune de manière telle que la pâte lavée provenant du côté sortie de l'une ou plusieurs des unités de lavage est transportée vers un réservoir de retenue, que la xylanase ayant une activité et une stabilité à pH élevé et une stabilité à température élevée est ajoutée directement en amont du réservoir de retenue, et que la pâte traitée à l'enzyme passe plus loin dans le procédé vers l'unité de lavage suivante.

2. Appareil pour mettre en oeuvre le procédé selon la revendication 1, caractérisé en ce qu'un réservoir de retenue ayant une tuyauterie munie d'accessoires destinés à l'introduction d'une enzyme est introduit en aval d'une ou de plusieurs des unités de lavage à l'exception de la dernière unité de lavage, en ce que tuyauterie est prévue pour transporter la pâte à papier vers le réservoir de lavage suivant, et en ce que l'unité de traitement à l'enzyme habituel située en aval de l'unité de lavage est abandonnée.
